# EUROPEAN PATENT SPECIFICATION

(11) **EP 0 165 345 B1**
(45) Date of publication and mention of the grant of the patent: **23.08.1989**
(21) Application number: 84304074.2
(22) Date of filing: 16.06.1984
(51) Int. Cl.: D06N 3/00, D06P 3/24, D06N 3/14

(54) **Grained artificial leather having good colour fastness and dyeing method of ultrafine polyamide fibers**
Narbenkunstleder mit einer guten Farbechtheit und Verfahren zum Färben von ultrafeinen Polyamidfasern
Cuir artificiel grainé ayant une bonne solidité de la couleur et procédé de teinture de fibres en polyamide ultrafines

(43) Date of publication of application: 27.12.1985
(62) Divisional of application: 87117815.8
(73) Proprietor: TORAY INDUSTRIES, INC., Tokyo 103 (JP)
(72) Inventor: Nishikawa, Toshio, Koga-Gun Shiga-Ken (JP); Imai, Shio, Otsu-shi Shiga-Ken (JP); Yagi, Kenkichi, Otsu-shi Shiga-Ken (JP); Yoshida, Yuriko, Otsu-shi Shiga-Ken (JP); Shimada, Masato, Otsu-shi Shiga-Ken (JP); Nagashima, Junnosuke, Kusatsu-shi Shiga-ken (JP); Nakamura, Teruo, Otsu-shi Shiga-Ken (JP)
(74) Representative: Dealtry, Brian

(56) References cited:
- EP-A- 0 038 202
- DE-A- 2 731 291
- DE-A- 3 314 478
- FR-A- 2 401 766
- US-A- 3 899 292
- CHEMICAL ABSTRACTS, vol. 94, no. 4, January 1981, page 46, abstract 16727u, Columbus, Ohio, US; & JP - A - 80 98 974 (KURARAY CO., LTD.) 28-07-1980
- JAPANESE PATENTS GAZETTE, week 8349, 25-01-1984, page 7, Derwent Publications, London, GB; & JP - A - 58 186 684 (KURARAY K.K.) 19-04-1982
- CHEMICAL ABSTRACTS, vol. 95, no. 14, October 1981, page 76, abstract 117007k, Columbus, Ohio, US; & JP - A - 81 73 167 (TORAY INDUSTRIES, INC.) 17-06-1981
- CHEMICAL ABSTRACTS, vol. 84, 1976, page 78, abstract 6403q, Columbus, Ohio, US; & JP - A - 75 100 383 (KANEBO LTD.) 08-08-1975
- CHEMICAL ABSTRACTS, vol. 96, no. 18, Mai 1982, page 82, abstract 144370a, Columbus, Ohio, US; J. GUTHRIE: "The effect of tanning agents on the rate of alkaline desorption of acid dyes from nylon 6", & COLOURAGE 1982, 29(4), 3-9
- JAPANESE PATENTS REPORT, vol. U, no. 35, page 12, Derwent Publication, London, GB; & JP - B - 73 28 041 (KURARAY)
- JAPANESE PATENTS REPORT, vol. 81, no. 9, 27-03-1981, pages 2,3, Derwent Publications, London, GB; & JP - B - 81 008 128 (TORAY INDS)

## Description

The present invention relates to a grained artificial leather having good colour fastness and to a process for dyeing ultrafine polyamide fibers into deep, bright colours, keeping good colour fastness to dry cleaning in charged system.

The grain layer of conventional artificial leathers are made by providing a porous or/and nonporous layer of a resin such as polyurethane on porous sheets made of elastomeric polymers and a fiber base such as woven, non-woven or knitted fabrics. However, such resins do not show good dyeability and colour fastness, especially when subjected to dry cleaning processes.

Therefore, dope dyeing has been applied to the resins of grained surface. However, dope dyeing is not suitable for manufacturing small quantities of artificial leathers of many colours. Further, the appearance of artificial leathers which are dope dyed is monotonous and opaque due to lack of transparency and lusters.

On the other hand, Japanese Patent Publication No. 28041/1973, teaches that some kinds of polyurethane whose soft segment is polyethyleneglycol (PEG-type PU) can be dyed with a metal complex dye. However, artificial leathers comprising PEG-type PU and a fiber base of ultra-fine fibers have no great practical value because they do not have good colour fastness as a whole, owing to an insufficient colour fastness of the ultra-fine fibers. Further, when the fiber base is impregnated or coated with porous resins, the porous resins, exhibit poor colour fastness when exposed to dry cleaning and spoil the appearance, not only of the back surface but also, of the grain surface of the artificial leather. The faded porous polyurethane effect even appears through the dyed grained surface.

On the other hand, a number of proposals have been made as to leather-like fabrics made of ultrafine fibers, such as suede-like, nubuk-like, woven or knitted fabrics, as well as grained artificial leathers. And, now, extra ultrafine fiber around or less than 0.01 denier (about 1.11 x 10-³ tex) is attracting our interests to obtain a softer hand or a more dense appearance.

However, as fibers become more fine, dyeing deeply and brightly become more difficult because of increased surface reflection of the extra fine fibers.

For example, though polyamide fibers such as nylon-6 and nylon-66 have such advantages over polyester fibers as softness, high wear resistance and brightness of colour, the use of polyamide ultrafine fibers for clothing has been delayed so far because dyes are very liable to come off in washing and dry cleaning.

Japanese Patent Publication No. 8128/1981 mentions the attempts to improve colour fastness by increasing molecular orientation of the ultrafine nylon fibers. However their colour fastness is insufficient when exposed to dry cleaning in which charge soap is used. Extra-ultrafine fibers around or less than 0.01 (about 1.11 x 1 0-3 tex) denier always show complete fading of colour even if they are dyed with the dyes said to give highest colour fastness to fibers of ordinary thickness.

Though thren-type vat dyes (vat dyes deriva- tived from anthraquinone), whose colour fastness is best amongst other dyes, can be also applied to the composite sheet of ultrafine polyamide fiber and polyurethane (Laid-Open Japanese Patent Application Publication No. 1365/1980), they can neither give any heavy sheds nor show good resistance to the synthetic solvents used in dry cleaning. Further, not only do they cause photo- tendering for some hues, but also the strong base used in the dyeing process leads to deterioration of the polyurethane.

The object of this invention is to provide a dyeable artificial leather, particularly a dyeable grained artificial leather, having good colour fasteness, bright, deep colours, excellent lusters, soft hand and high durabilities. The object can be achieved, most preferably by dyeing an artificial leather comprising a super-entangled ultrafine fiber base and PEG-type PU applied thereon with a metal dye complex.

In one aspect the invention provides a grained artificial leather dyed with metal dye complexes and an applied fixing agent, comprising a fiber base of ultrafine polyamide fibers and/or bundles thereof of which, at a surface providing a grained surface, the fibers or bundles thereof are super-entangled, the grained surface further comprising a polyurethane applied on the super-entangled surface wherein the soft-segment constituents of the polyurethane contains at least 5% by weight of polyoxyethylene chain having molecular weight of 500-5,000.

In another aspect the invention provides a process for manufacturing grained artificial leather, which comprises at least the following steps (1) to (5):
(1) making a fiber sheet being mainly comprised of ultrafine polyamide fibers of less than 22.2x10-³ tex or ultrafine polyamide fiber formable fibers,
(2) entangling said fiber sheets by applying high-velocity fluid streams to at least one surface thereof to provide a super-entangled surface,
(3) applying a polyurethane to said super-entangled surface to provide a grain surface, wherein the soft-segment constituents of the polyurethane contain at least 5% by weight of polyoxyethylene chain having molecular weight of 500-5,000,
(4) dyeing said sheet comprising a fiber base and applied polyurethane with at least one dye selected from the group consisting of metal dye complexes, and
(5) applying a fixing agent.

Suitably in one process according to the invention the fixing agent is selected from the group consisting of tannins, synthetic tannins and their derivatives, or tannin and metal; tannins and metal salt are used as fixing agents in another process.

The dyeing method makes it possible to provide deep and bright colours whilst maintaining sufficient colour fastness to enable dry cleaning of the extra-ultrafine polyamide fibers.

It is preferable for the facility of processing and handling to convert ultrafine fiber formable fibers into ultrafine fibers or bundles thereof at an appropriate stage. They can however be manufactured directly by methods such as wet spinning, super-drawing or melt-blow spinning.

Ultrafine fiber formable fibers include the chrysanthemum-like cross-section fibers in which one component is radially sandwiched between other components, multi-layered bicomponent fibers, radially multi-layered bicomponent hollow fibers, and islands-in-sea type composite fibers having fixed or unfixed cross section along the fiber axis. They may be used by mixing more than two of the fibers.

For obtaining leathers having soft hand and smooth surface, the thickness of the ultrafine fibers which can be obtained from the ultrafine fiber formable fibers should be less than 0.2 deniers (about22.2x 10⁻³tex), preferably less than 0.05 denier (about 5.55x 10-³ tex), more preferably less than 0.01 denier (about 1.1x10⁻³ tex).

As materials for the ultrafine fibers, polyamides such as nylon-6 and nylon-66, are preferable among others. Polyamides et even less than 0.01 denier (about 1.11x10⁻³ tex) can be deeply coloured with good colour fastness by the dyeing method stated later.

As binding components (sea components) for ultrafine fiber formable fibers, those readily-separable type ultrafine fiber components or those different in the solubility are selected. For the facility of spinning and removal, polystyrene, polyethylene; their copolymers, and copolymerized polyesters are preferably used. Particularly the copolymers of styrene with acrylic acid and/or methacrylic acid are preferable amongst them for obtaining strong fibers due to easiness of applying a high drawing ratio.

In this invention, to improve colour fastness, it is preferable to increase drawing ratio to achieve high molecular orientation or high degree of crystallinity. Drawing ratio more than 2.0 times, preferably more than 2.5 times, are usually preferable, provided the spinning speeds of 600 to 1,500 m/min. (10 to 25 m/second) are used.

The ultrafine fibers of the grained surface should preferably have a size less than 0.2 denier (about 22.2x10⁻³tex). If not, a smooth grained surface is difficult to form because the excessive fiber stiffness affects their smoothness, the surface can produce unsightly creases and cracks, and crumpling readily causes cracks and surface unevenness. The ultrafine fibers of less than 0.2 denier (about 22.2x 10-³ tex), preferably of less than 0.05 denier (about 5.55x 10-³ tex), more preferably of less than 0.01 denier (about 1.11 x10⁻³ tex) can be densely entangled so that a surface which is highly smooth, flexible, and not liable to cause cracks, and has a soft touch feeling is obtainable.

The fiber structure of or just beneath the grained surface has ultrafine fibers and/or their bundles, mutually super-entangled. They should preferably be such that the distance between the fiber entanglement points (defined later) is less than 200 micrometers. The fiber structures with less entanglement such as entangled only by needle punching are not preferable because they are apt to fluff or crack when subjected to friction, crumpling, or repeated shearing or bending. Such fiber bases require reinforcement with a great quantity of porous resins to maintain their strength and dimensional stability and, consequently, such sheets are poor in dyeing fastness. Forthe purpose of reducing the amount, of porous resins for eliminating such defects, the distance between the fiber entanglement points should preferably be less than 200 micrometers or more preferably less than 100 micrometers.

The term "the distance between the fiber entangelement points" is defined in Laid-Open Japanese Patent application Publication No. 191280/1983 (Tokkai-sho 58-191280).

A short average distance between points of entanglement produces a high density of entanglement.

The average distance between the fiber entanglement points is measured in the following manner. When observed from the surface with a scanning electron microscope, the fibers are considered to form an entanglement point when an upper fiber which has passed over and across a lower fiber then passes under and across another fiber. It will be assumed that the constituent fibers are f₁, f₂, f₃, ..., the point at which two fibers f₁ and f₂ are entangled with each other is a, and another point at which the upper fiber f₂ is entangled with another fiber with the fiber f₂ being the lower fiber is a₂ (the entanglement point between f₂ and f₃). Similarly, the entanglement points a3, a4; a₅, ... are determined. The linear distances a,a₂, a₂a₃, a₃a₄, a₄aₛ, aₛaₑ, aₑa₇, a₇a₃, a₃aₐ, a₈a₇, a₇ag, a₉a₆, ... measured along the surface are the distance between the fiber entangling points and their average is taken.

In the present invention, the fibers of the surface portion preferably have an average distance between the fiber entangling points of less than about 200 micrometers as measured by this method. In fiber structures where the average distance between the entangling points is greater than about 200 micrometers, such as in those fiber structures in which the entanglement of the fibers is effected only by needle punching, only little entanglement of the fibers occurs.

If fiber entanglement is so dense that the distance between its points is less than 200 micrometers, the amount of polyurethanes applied thereto can be decreased. Namely it is possible to decrease porous polyurethane to be impregnated in the fiber base or to decrease the thickness of polyurethane layer applied to the surface. The fomer spoils colour fastness and the latter spoils soft hand and delicate appearance. The fiber base may be nonwoven, laminated nonwoven or woven or knitted fabrics laminated and entangled with a nonwoven. Amongst them, a nonwoven fiber base comprising a surface portion of super-entangled ultrafine fibers and/or their bundles, said ultrafine fibers and/or their bundles being branched from the ultrafine bundles of the inner portion, is most preferable. It is preferable that the degree of branching and entanglement vary at the boundary between the surface and inner portions. By applying water jet streams to the ultrafine formable fiber sheet, entanglement and branching often occur throughout its thickness. The dense entanglement and branching around the surface portion brings about the sheet a smooth surface and excellent stability such as against fluff and deformation. Looser entanglement than the surface of the inner portion brings about softness to the sheet.

The amount of resin depends on the intended purposes for the leather. For clothing, however, it should preferably be Oto 50% and more preferably less than 20% based on the fiber weight.

The resins used for the grain layer in accordance with the invention are required to be the urethane polymers having at least 5% by weight of polyoxyethylene chains with molecular weights of 500 to 5,000 based on total weight of the soft segment. If the amount of polyoxyethylene chains is less than 5% by weight, bright colours are difficult to obtain by dyeing. The molecular weight of polyoxyethylene chains is required to be 500 to 5,000 for keeping the softening temperature, resistance to flexing and solvent within their practicable range.

Polyurethanes whose soft segment contains polyoxyethylene chains should preferably be dyed with anionic dyes such as metal dye complexes, acid dyes and reactive dyes because they are highly affinitive thereto and particularly dyeable with metal dye complexes and have good colour fastness.

They may of course be blended or copolymerized with a proper quantity of another polyether polyester and copolymerized polyesters for improving mechanical strength.

Polyurethane polymers in accordance with the invention are not limited to linear type and may be the cross-linked type such as cross-linked with hexamethylene diisocyanate trimer. Cross-linked polyurethanes generally improve resistances to scratch, scuff, organic solvent and hot water, but is defective in flex resistance. However, in the present invention, flex resistance is much improved by virtue of super-entangled surface structure.

The soft segment of the polyurethane may be polyoxyethylene glycol alone, but may also be its mixtures with polyether diols such as polyoxyp- roplyeneglycol, polyoxytetramethyleneglycol and polyester diols such as polyethyleneadipate, poly- butyleneadipate, polyhexamethyleneadipate and polycaprolactone, and copolymers thereof.

PEG-type PU may be mixed with other polyurethanes so that the amount of polyoxyethylene segments is more than 5% by weight based on the total weight of the soft-segment.

Organic diisocyantes used to make the polyurethane include aromatic ones such as diphenylmethane-4,4'-diisocyanate, aromatic-aliphatic ones such as xylylenediisocyanate, aliphatic diisocyanates such as hexamethylenediisocyanate, and alicyclic ones such as isophoronediisocyanate and hydrogenated diphenylmethane-4,4'-diisocyanate. Amongst them, aromatic diisocyanates, particularly diphenylmethane-4,4'-diisocyanate, is preferable for obtaining good physical characateristics such as thermal stability, solution stability and fracture strength.

Alicyclic diisocyanates such as isophorone ones are preferably for obtaining anti-yellowed (not easily coloured even when exposed to sun) type polyurethanes.

Chain extenders for the polyurethane include water, low-molecular diols such as ethyleneglycol and propyleneglycol, aromatic diamines such as ethylenediamine, aliphatic diamines such as 4,4'-diaminodiphenylmethane, alicyclic diamines such as 4,4'-diaminodicyclohexylmethane and isophoronediamine, alkanolamines such as ethanolamine, hydrazines, and dihydrazide such as succinic one. Amongst them diamine compounds are preferable and 4,4'-diaminodiphenylmethane is particularly preferable for practical use because of its heat resistance and 4,4'-diaminodicyclohexylmethane is more preferable for light resistance. They may of course be used along or in combination.

The polyurethanes are generally manufactured in the presence of solvents. Suitable solvents are dimethylformamide, (referred to DMF hereinunder), dimethylacetamide, ethylacetate and toluene. Amongst them DMF should be preferable used. Elastomers other than polyurethane such as polyamide, polyester, polyvinyl chloride, polyacrylic ester copolymers, neoprene, styrenebutadiene copolymers, acrylonitrile-butadiene copolymers, polyamino acid, polyamino acid- polyurethane copolymers, and silicone resins may be mixed with the polyurethanes, and if necessary may be applied in lessthan 10 microns thickness to the grained surface of the present invention. As a matter of course, plasticizers, fillers, stabilizers, crosslinking agent and so forth may be added thereto.

When flexibility and soft feeling are particularly demanded, the resin should be applied in great quantities to the uppermost very-thin portion of the grained surface and not at all or in small quantities to the other parts.

The deep luster and bright colour are obtainable by dyeing the leathers, with one or more dyes selected from anionic dyes which have a negative charge in aqueous solution such as metal dye complexes, acid dyes and reactive dyes. Further, when polyamide ultrafine fibers are used, the dyeing method described later is particularly preferable for obtaining heavy shade, and high colour fastness.

The colour of the urethane polymers may be improved by preliminarily adding dyes and/or pigments thereto.

For making ultrafine fibers, islands-in-sea type fibers are representative. It is produced, for example, by using a spinning system mentioned in Japanese Patent Application Publication No. 18369/1969 (Tokko-sho 44-18369) or dope mixed spinning. Usually ultrafine fiber formable fibers are cut into short fibers, crimped with stuffing box, formed into web and subjected to needle punching. Or, continuous filaments are spread into sheet without cutting and subjected to needle punching. Further the ultrafine fiber formable fibers may be placed on and entangled with other nonwoven, woven knitted fabrics. After that or occasionally without needle-punching, high-velocity fluid streams are applied to the sheet. Water is most preferably used amongst other fluids. The branching and entanglement of the fibers are achieved through the treatment. The ultrafine fiber formable fibers may be converted into bundles of ultrafine fibers before treatment with high pressure fluid streams. In such a case, the pressure of the fluids may be 5--100 kg/cm² (about 4.9-98 Bar).

Even before conversion, a similar pressure may be applied for easy separable fibers. However, 100-300 kg/cm³ (about 98-294 Bar) is preferable for the fibers not liable to separation. The degree of branching and entanglement can also be changed by contact times. Pressure may be changed each time of contact. The degree of ultrafining can be controlled by treating the fiber sheets with solvents for at least a part of components. The dissolution of part of the fibers can be carried out even after impregnating or coating with resins. In this case, products become softer because many spaces where the part of components were formed along the fiber axis in the products.

The resin solution or dispersion for the grained surface may be applied by reverse roll coater, gravure coater, knife coater, slit coater, spraying and other methods. The coated surface is pressed and if necessary heated for smoothing or embossing the surface. Sometimes pressing the fiber sheets before coating the resin is also effective for improving smoothness.

In this invention, heavy shade, high colour fastness of polyamide ultrafine fibers is attainable through the colour fixing after dyeing with metal dye complexes.

Generally speaking, polyamide fibers such as nylon-6, can be dyed beautifully with acid dyes, disperse dyes or metal dye complexes. However, ultrafine polyamide fibers less than 0.2 denier (about 22.2x 10-³ tex) is inferior to ordinary fibers in colour fastness. This trend is remarkable for as extra-ultrafine fibers with less than 0.01 denier (about 1.11 x 1 0-3 tex).

We found that the ultrafine polyamide fibers can be deeply dyed using metal dye complexes such as mordant dyes, acid mordant dyes, 1:1 metal-complex dyes, 2:1 pre-metallized dyes and metal complex direct dyes of molecular weights more than 700, more preferably of more than 900. The methods for this dyeing include dip drying, pad steam drying and pad drying and are not limited. Amongst the dyes, 2:1 premetallized dyes of larger molecular weights are easy to be produced. We also found that the ultrafine fibers of less than 0.01 denier (about 1.11x10⁻³ tex), particularly with 0.001 denier (about 0.111 x 1 0-3 tex), can unexpectedly be dyed with so-called Irgaran- type metal complex dyes having low hydrophilicity groups such as sulfonamide and sulfon- methyl groups.

The metal dye complexes enhance dye bonding with the fibers by forming complex salts between the dye molecules and chrome or other metal atoms and can provide ordinary fibers with good colour fastness but in ultrafine fibers almost all colour fade by dry cleaning with charge-soap containing synthetic solvents.

We, however, discovered that remarkable effects are obtained by fixing synthetic tannins and tannic acid derivatives (synthetic and natural) or tannins and metal salts in combination after dyeing with metal dye complex dyeing. The fixing after dyeing with metal dye complexes has been said to be neither effective nor necessary for ordinary fibers at all. However, the fixing with tannins and metal salts ensures good colour fastness even to the extra ultrafine fibers in dry cleaning with synthetic solvents (such as per- chlene which is said to have the strongest cleaning power).

Term "tannins" in accordance with the invention is generically given to hydrolysable tannins, condensed tannins and the complex tannins which has both properties. They are contained in the barks, leaves, roots and fruits of plants. Preferable tannins amongst them are gallotannins (tannic acid) classified in the category of hydrolytic tannins that are represented by Chiness gallotannin and gallic acid.

The metal salts in accordance with the invention include antimony complex salts,. iron salts, chrome salts, copper salts, bismuth salts and their complex compounds. Preferable amongst them is potassium antimonyl tartrate in the category of antimonide complex compounds.

Such fixing methods may be conducted by continuous 2-bath process or may be carried out by separate 2-bath process, namely, impregnation with tannins solution, drying the impregnated sheet, impregnation with metal salts solution and drying, in this order. In the former, temperature can be set at 25 to 100°C. Too low temperatures lower the solubility and adsorbability of the fixing agent. On the contrary, too high temperature causes dissolving out of the absorbed dye into the treating solutions. Temperatures of 40 to 85°C, particularly 50 to 80°C, are therefore preferable and result in satisfactory fixing effects.

The mechanism of fixing is not known in detail, but it can be assumed that a layer of the fixing agent is formed on the surface of the ultrafine fibers and the layer multiplicatively enhances the affinity between the dyes and fibers so that dyes become difficult to move. Though such fixing treatment tends to harden the sheets, it is however also amazing that the above effects are kept even after finishing through mechnanical crumpling.

Such crumpling methods are not limited and include dry heat mechanical crumpling and wet heat and hot water tumbler crumpling. Further it can be carried out simultaneously with the fixing by using liquid flow dyeing machines.

The fiber sheets thus obtained may be futher subjected to washing and finishing agent treatment, if necessary, after the dyeing and fixing. Further the addition of polyurethanes or raising such as buffing can be applied either before or after the dyeing and fixing. Surface active agent treatment is preferable for dyeing the fiber sheets impregnated with high-molecular elastomer other than PEG-type PU. That is, because other type polyurethanes suitable for impregnation are extremely inferior in colour fastness, it is rather preferable to preliminarily remove the dyes absorbed to the impregnated elastomers with surface active agents.

Amongst such surface active agents, anionic, nonionic and amphoteric surfactants are effective. Particularly the latter two are preferable. Particularly preferable amongst them are polyoxyalkylene nonionic and betaine amphoteric surface active agents. The former include polyoxyal- kylenealkylamine, polyoxyethylenealkylether, polyoxyethylenealkylarylether, polyoxyethylenealkylether, polyoxyethylenealkylester, poly- oxyethylenealkylamide, polyoxyethylenepolyox- ypropylene, polyoxyethylenealkylphenol and polyoxyethylenephenylether for example.

When the fiber sheets are prepared with the multi-layered ultrafine fiber formable fibers made of polyamide and the products are subjected to multi-colour dyeing, a melange coloured product having good colour fasteness can be obtained.

### Example 1

A staple of island-in-sea type fiber (4 denier (about 0.444 tex), 51 mm length) having 7 islands, each islands consist of many islands-in-island (I-I-I) and a sea-in-island (S-I-I), was obtained by spinning at a speed of 1,200 m/min (about 20 m/ sec), drawing at 2.6 times, being subjected to crimping and cutting. The islands-in-sea type fiber is composed of 65 parts of acrylic acid- styrene copolymer (referred to as AS resin hereinunder) as the sea and the S-I-I component and 35 parts of nylon-6 as I-I-I component. The average thickness of the I-I-I was 0.002 denier (about 0.222x10 tex).

A web was formed through card, cross-lapper and needle-punched with single barbed needles for entanglement. The sheet has a weight 430 gr./ m², an apparent density of 0.17 gr./cm³ and an average distance between the entanglement points of 378. Both surfaces of the sheet were treated one time respectively with high-velocity fluid streams of 100 kg/cm² (about 98 Bar) pressure from a nozzle having 0.25 mm diameter holes arranged in one row at 2.5 mm intervals, while oscillating the nozzle. The nonwoven sheet thus obtained showed the super-entangled structure in which the islands-in-sea type fibers were branched into extra ultrafine fibers and/or their bundles, and the average distance between the fiber entanglement points was 56 micrometers at the surface.

Next the nonwoven sheet was shrunk in 85°C hot water, dried and smoothed between rubber roll and hot iron roll having smooth surface.

A prepolymer obtained from polyoxyethyleneglycol of molecular weight of 600 and isophoronediisocyanate was chain extended with 4,4'-diaminodicycylhexylmethane, terminated at the end with ethanolamine and cross-linked with 15 parts of a hexamethylenediisocyanate trimer. Then the cross-linked polyurethane was coated with gravure coater, on the smoothed surface. The amount of coating was 5 gr./m². The coated surface was pressed with a hot emboss roll, for embossing and integrating the coated resin with the super-entangled surface.

Thereafter AS resin was almost completely removed with trichloroethylene and the islands-in-sea type fibers were ultrafined.

A sheet thus obtained was subjected to dyeing and fixing using a wince dyeing machine under the following condition.

### Dyeing:

Dye stuff: Iregalan Black GBL 200%, 10% owf.

Dyeing temperaturextime: 98°Cx60 min.

### Fixing:

Fixing agents: tannic acid and tartar emetic.

Treating method: treatment with weakly acidic bath containing 10% owf tannic acid at 50°C, for 50 min, and,

treatment with weakly acidic bath containing 5% owf tarter emetic at 50°C, for 50 min.

Next, after adding a finishing agent, the sheet was softened with a tumbler crumpling machine and dried.

Both the grained surface and the reverse surface of thus-obtained sheet were colored dark black. It showed a softness free from undesirable rubber-like feeling and the grained surface has deep luster, resistances against scuff and repeated bending. Its washing and dry cleaning fastness according to JIS-L0844 L0860 (2% charge soap content) was good.

### Comparator Example 1

A grained artificial leather was obtained according to the same manner except using anti-yellowed (not easily coloured even when exposed to sun light) type polyester polyurethane instead of the PEG-type PU.

It showed a natural leather-like appearance as that of Example 1. However the grained surface was dyed into dark-blue not into dark black. Further, the colour of the grained surface was seriously faded by dry cleaning containing 2% charge soap.

### Comparative Example 2

The same needle-punched sheet as example 1 was immersed in a 15% aqueous solution of polyvinyl alcohol (referred to PVA hereinafter) at 85°, shrunk simultaneously, dried, impregnated with a 10% DMF solution of polyester polyurethane, coagulated with 30% DMF aqueous solution and sufficiently washed in 80°C hot water for removing PVA and DMF.

Next, the sheet was subjected to the surface smoothing with a hot roll and the same treatment as Example 1. The sheet showed unevenly coloured lines or portions like stood veins along ultrafine fiber bundles, and cracks arised during the dyeing, and ultrafine fibers were exposed therefrom. Further it had hard touch, unbright colour and feeling not natural leather-like as compared with Example 1.

Further when picked up by fingers, so bent as to have an acute angle, and rubbed against a thigh part of trousers with a large pressure applied, the Comparative Example 2 leathers showed peeled grained surface and exposed raising while the leather of Example 1 did not change in appearance at all.

## Claims

1. A grained artificial leather dyed with metal dye complexes and an applied fixing agent, comprising a fiber base of ultrafine polyamide fibers and/or bundles thereof of which, at a surface providing a grained surface, the fibers or bundles thereof are super-entangled, the grained surface further comprising a polyurethane applied on the super-entangled surface wherein the soft-segment constituents of the polyurethane contain at least 5% by weight of polyoxyethylene chain having molecular weight of 500-5,000.

2. A grained artificial leather according to Claim 1, wherein said ultrafine fibers and/or bundles thereof are branched from ultrafine fiber bundles or ultrafine fiber formable fibers located in the inner portion of the fiber base.

3. An artificial leather according to Claim 1 or 2, wherein the inner portion of the fiber base contains substantially no resin.

4. A process for manufacturing grained artificial leather, which comprises at least the following steps (1) to (5):
(1) making a fiber sheet being mainly comprised of ultrafine polyamide fibers of less than 22.2x10-³ tex or ultrafine polyamide fiber formable fibers,
(2) entangling said fiber sheets by applying high-velocity fluid streams to at least one surface thereof to provide a super-entangled surface,
(3) applying a polyurethane to said super-entangled surface to provide a grain surface, wherein the sogft-segment constituents of the polyurethane contain at least 5% by weight of polyoxyethylene chain having molecular weight of 500-5,000,
(4) dyeing said sheet comprising a fiber base and applied polyurethane with at least one dye selected from the group consisting of metal dye complexes, and
(5) applying a fixing agent.

5. A process according to Claim 4, wherein said fixing agent is selected from the group consisting of tannins, synthetic tannins and their derivatives.

6. A process according to Claim 4, wherein tannin and metal salt are used as fixing agents.

7. A process according to Claim 4, wherein said metal dye complex has molecular weight more than 700.

8. A process according to Claim 4, wherein said metal dye complex is a 2:1 premetallized dye.

9. A process for manufacturing an artificial leather according to Claim 4, wherein a crumpling is carried out after said dyeing.

## Patentansprüche

1. Marmoriertes Kunstleder, das mit Metallfarbstoffkomplexen gefärbt und auf das ein Fixativ aufgebracht ist, aus einer Fasergrundlage aus ultrafeinen Polyamidfasern und/oder Bündeln derselben, die an einer eine marmorierte Oberfläche liefernden Fläche superverschlungen sind, wobei auf die marmorierte Oberfläche mit den Superverschlingungen ein Polyurethan, dessen Weichsegmentbestandteile mindestens 5 Gew.-% einer Polyoxyethylenkette eines Molekulargewichts von 500-5000 enthalten, appliziert ist.

2. Marmoriertes Kunstleder nach Anspruch 1, dadurch gekennzeichnet, daß es sich bei den ultrafeinen Fasern und/oder deren Bündeln um Verzweigungen von im Inneren der Fasergrundlage befindlichen ultrafeinen Faserbündeln oder ultrafeine Fasern bildenden Fasern handelt.

3. Kunstleder nach Anspruch 1 oder 2, dadurch gekennzeichnet, daß das Innere der Fasergrundlage praktisch kein Harz enthält.

4. Verfahren zur Herstellung eines marmorierten Kunstleders, gekennzeichnet durch mindestens folgende Stufen (1) bis (5):
(1) Herstellen einer Faserlage, die hauptsächlich aus ultrafeinen Polyamidfasern von weniger als 22,2x10-³ tex oder ultrafeine Polyamidfasern bildenden Fasern besteht;
(2) Verschlingen der Faserlagen durch Einwirkenlassen von Hochgeschwindigkeitsfluidumströmen auf mindestens eine ihrer Oberflächen zur Ausbildung einer superverschlungenen Oberfläche;
(3) Aufbringen eines Polyurethans, dessen Weichsegmentbestandteile mindestens 5 Gew.-% einer Polyoxyethylenkette eines Molekulargewichts von 500-5000 enthalten, auf die superverschlungene Oberfläche zur Ausbildung einer marmorierten Oberfläche;
(4) Anfärben der Lage aus einer Fasergrundlage und dem applizierten Polyurethan mit mindestens einem Metallfarbstoffkomplex und
(5) Aufbringen eines Fixativs.

5. Verfahren nach Anspruch 4, dadurch gekennzeichnet, daß das Fixativ aus Tanninen, künstlichen Tanninen und deren Derivaten ausgewählt ist.

6. Verfahren nach Anspruch 4, dadurch gekennzeichnet, daß als Fixative Tannin und en Metallsalz verwendet werden.

7. Verfahren nach Anspruch 4, dadurch gekenzeichnet, daß der Metallfarbstoffkomplex ein Molekulargewicht von über 700 aufweist.

8. Verfahren nach Anspruch 4, dadurch gekennzeichnet, daß es sich bei dem Metallfarbstoffkomplex um einen 2:1 vormetallisierten Farbstoff handelt.

9. Verfahren zur Herstellung eines Kunstleders nach Anspruch 4, dadurch gekennzeichnet, daß nach dem Anfärben eine Knitterbehandlung durchgeführt wird.

## Revendications

1. Cuir artificiel grainé teint avec des complexes métalliques teignants et un agent de fixation appliqué, comprenant une base de fibres en fibres ultrafines de polyamide et/ou des fasiceaux de telles fibres dans lesquels, sur une surface présentant une surface grainée, les fibres ou les faisceaux de fibres sont super-emmêlés, la surface grainée comprenant en outre un polyuréthane appliqué sur la surface super-emmêlée, dans lequel les constituants à segment souple du polyuréthane contiennent au moins 5% en poids d'une chaîne polyoxyéthylène ayant un poids moléculaire de 500 à 5000.

2. Cuir artificiel grainé selon la revendication 1, dans lequel lesdites fibres ultrafines et/ou les faisceaux de ces fibres sont ramifiés à partir de faisceaux de fibres ultrafines ou de fibres pouvant être formées en fibres ultrafines, situées dans la partie interne de la base de fibres.

3. Cuir artificiel selon la revendication 1 ou 2, dans lequel la partie interne de la base de fibres ne contient pratiquement aucune résine.

4. Procédé de fabrication de cuir artificiel grainé, comprenant au moins les opérations (1) à (5) suivantes:
(1) fabrication d'une feuille de fibres constituée principalement de fibres ultrafines de polyamide, de moins de 22,2x10-³ tex, ou de fibres de polyamide pouvant être formées en fibres ultrafines;
(2) emmêlement desdites feuilles de fibres en appliquant des jets fluides à grande vitesse sur au moins une surface desdites feuilles pour obtenir une surface super-emmêlée;
(3) application d'un polyuréthane sur ladite surface super-emmêlée pour obtenir une surface grainée dans laquelle les constituants à segment souple du polyuréthane contiennent au moins 5% en poids d'une chaîne de polyoxyéthylène ayant un poids moléculaire de 500 à 5000;
(4) teinture de ladite feuille comprenant une base de fibres et du polyuréthane appliqué sur cette base au moyen d'au moins un colorant teignant choisi dans le groupe consistant en des complexes métalliques teignants, et
(5) application d'un agent de fixation.

5. Procédé selon la revendication 4, dans lequel ledit agent de fixation est choisi dans le groupe comprenant les tanins, les tanins synthétiques et leurs dérivés.

6. Procédé selon la revendication 4, dans lequel on utilise comme agents de fixation un tanin et un sel métallique.

7. Procédé selon la revendication 4, dans lequel ledit complexe métallique teignant a un poids moléculaire supérieur à 700.

8. Procédé selon la revendication 4, dans lequel ledit complexe métallique teignant est un colorant prémétallisé à 2:1.

9. Procédé fabrication d'un cuir artificiel selon la revendication 4, dans lequel on pratique une opération de froissage après ladite opération de teinture.
